# EUROPEAN PATENT SPECIFICATION

(11) **EP 3 507 413 B1**
(45) Date of publication and mention of the grant of the patent: **19.07.2023**
(21) Application number: 16759771.5
(22) Date of filing: 01.09.2016
(51) Int. Cl.: D06M 15/285, D06M 15/431

(54) **FLAME RETARDANT TREATED FABRICS WITH LOW FORMALDEHYDE CONTENT**
MIT FLAMMSCHUTZMITTEL BEHANDELTE GEWEBE MIT GERINGEM FORMALDEHYDGEHALT
TISSUS TRAITÉS PAR IGNIFUGEANT À FAIBLE TENEUR EN FORMALDÉHYDE

(43) Date of publication of application: 10.07.2019
(73) Proprietor: Energy Solutions (US) LLC, Princeton, NJ 08540 (US)
(72) Inventor: WOODWARD, Gary, Northwich Cheshire CW9 5QR (GB); HAND, Geoffrey, Hakesowen West Midlands B62 8TA (GB); HICKLIN, Robert, Ashby de la Zouch Leicestershire LE65 2QB (GB); SEABROOK, Matthew, Oldbury West Midlands B69 4LN (GB)
(74) Representative: Osha Liang
(86) International application number: PCT/EP2016/070586
(87) International publication number: WO 2018/041351

(56) References cited:
- EP-A1- 0 451 664
- DE-B4-102006 040 075
- GB-A- 2 271 787
- US-A- 3 101 278
- US-A1- 2011 092 119
- US-B2- 9 493 398

## Description

The instant invention relates to textile articles comprising (or consisting in) a fabric treated by flame-retardant polymer polymer obtained from an ammonia curing of a condensate of (i) a tetrakis (hydroxyorgano) phosphonium salt (also referred as "THP⁺ salt") ; and (ii) urea and/or thiourea (herein referred as "(thio)urea") ; followed by an oxidation into phosphine oxide groups of at least one part of the phosphonium groups present on the cured condensate.

Flame retardant treatments of this type are well known and has been described e.g. in the European patent application EP 0 709 518. In these treatment, the fabric to be treated is generally impregnated with the condensate of the THP⁺ salt and (thio)urea (optionally together with an amine as described in EP 0 709 518, such as an aliphatic amine having 12 carbon atoms or more, such as n-dodecylamine; n-octadecylamine, n-hexadecylamine, and/or n-eicosylamine) and, typically, the fabric is then dried and then cured with ammonia (NH₃) whereby a phosphonium-based polymer is produced within the fibers of the fabric, which is mechanically fixed to the fabric. After the curing, the obtained polymer is oxidized in order to convert at least a part of the trivalent phosphorus (carried by the phosphonium group) into a pentavalent phosphorous (an phosphine oxide group). Examples of fabrics treated according to this process and textile articles and garments made thereof are those sold under the trademark PROBAN^{®}.

In the scope of the instant invention, the inventors have now found that a fabric treated according to the above-mentioned process tends to generate formaldehyde over the time. Concretely, in many cases, the free HCOH content increase with the time and, generally, becomes greater than 100 ppm or even greater than 300 ppm over a few years. The term "free HCOH content" as used in the instant description refers to the content of free formaldehyde (HCOH) in the fabric as measured according to the European standard No. EN ISO 14184-1.

This identified formation of formaldehyde constitutes a potential bar, because of the toxicity of formaldehyde. Especially, a fabric intended to be in contact with the human skin should have a very low content of HCOH, typically of less than 300 ppm, more preferably less than 200 ppm for an indirect contact (with another piece of clothes between the fabric and the skin) and of less than 100 ppm, preferably less than 75 ppm.

Flame retardant treatments with THP compounds are also disclosed in US-A-2011 0092119,GB-A-2271787, EP-A-451 664 and US-A-3101278 but the amount of free formaldehyde over the time is not discussed.

The instant invention aims at providing a flame retardant treatment process making use of the materials which lead to a low content of formaldehyde that remains low over the time.

To this end, the instant invention proposes to make use of the above mentioned process but in specific conditions, that have been found inhibit the formaldehyde formation over the time. Namely, the inventors have now surprisingly found that a limitation of the content of trivalent phosphorus (i.e. phosphorus of phosphonium groups by opposition of pentavalent phosphorus of the phosphine oxide groups >P=O) in the treated fabric leads to a strong decrease of the formation of formaldehyde.

Especially, the inventors have now shown that when a fabric has a content of trivalent phosphorous, i.e. of the phosphorus present in phosphonium groups, of less than 1% by weight based on the total weight of the flame-retardant treated fabric, then substantially no formaldehyde HCOH is generated over the time. The inhibition of the formation of HCOH is even more efficient when the content of trivalent phosphorous is lower than 0.9%, and even more when lower than 0.8%.

On this basis, according to a first aspect, one subject matter of the instant invention is a textile article, such as an item of clothing for example, comprising at least one flame-retardanttreated fabric including an oxidizedpolymer obtained from an ammonia curing of a condensate of (i) a tetrakis (hydroxyorgano) phosphonium salt; and (ii)urea and/or thiourea; followed by an oxidation into phosphine oxide groups of at least one part of the phosphonium groups present on the cured condensate,
wherein said flame-retardant treated fabric :
- is intended to be used as a stable substrate in which the formation of formaldehyde over the time is inhibited , for example for a long term contact with the skin ; and
- contains less than 1% by weight, preferably less than 0.9% by weight and even more preferably less than 0.8% by weight of phosphorus present in phosphonium groups (trivalent phosphorus), based on the total weight of the flame-retardant treated fabric.

In a textile article according to the invention, the molar ratio P3:P5 of the trivalent phosphorus (as present in the phosphonium groups) to the pentavalent phosphorus (as present in the phosphine amide groups) is typically of less than 60%, for example of about 50%. The total content of phosphorus in a fabric according to the invention is typically of around 2% based on the total weight of the flame-retardant treated fabric.

Another subject matter of the instant invention is a process for preparing the above mentioned textile article, comprising :
(a) a flame retardant treatment of the fabric, including :
   (a1) an impregnation of said fabric with the condensate of (i) a tetrakis (hydroxyorgano) phosphonium salt; and (ii) urea or thiourea (a2) a curing with ammonia of the impregnated condensate ;
   (a3) an oxidation of the polymer resulting from the curing, typically with H₂O₂
(b) an analysis of the content of the phosphonium groups in the fabric, followed by a repetition of the sequence of the steps (a3) and(b) if the analysis shows that the fabric contains 1% or more of phosphorus present in phosphonium groups, based on the total weight of the flame-retardant treated fabric.

Step (a3) may be followed by a washing of the oxidized fabric obtained in step (a3), typically by immersion within at least one (for example 2 or 3) washing bath, typically a water-containing washing bath.

In the process of the invention, step (b) comprises an analysis wherein the content of trivalent phosphorus is checked and adapted if needed. The analysis may for example be made by ³¹P NMR, that allows to distinguish a phosphonium peak at around 25 ppm and an amine oxide peak at around 47 ppm

If needed, the sequence of the steps (a3) and (b) are repeated many times until the sought trivalent phosphonium content is not below the sought value.

According to a specific embodiment, the sequence of the steps (a3) and (b) may be repeated even after having obtained a content below the sought value (for example if a very low content of trivalent phosphonium is sought.

According to a possible embodiment, in step (b), the analysis is followed by a repetition of the sequence of steps (a3) and (b) if the analysis shows that the oxidized polymer contains 0.9% or more of phosphorus present in phosphonium groups, based on the total weight of the flame-retardant treated ffabric

According to yet another aspect, the invention relates to the use of a flame-retardant treated fabric containing less than 1% by weight, preferably less than 0.9% by weight and even more preferably less than 0.8% by weight of phosphorus present in phosphonium groups (trivalent phosphorus), based on the total weight of the flame-retardant treated fabric, as a substrate stabilized against formation of formaldehyde, for example for a long term contact with the skin.

The expression "long term" contact with the skin, especially include a contact with the skin, preferably more than one year, more preferably more than 2 years, and even more preferably at least 3 years, after the synthesis of the oxidized polymer.

In the scope of the instant invention, the inventors have now shown that, in some specific conditions, step (a) systematically allows to obtain the sought content of trivalent phosphorous, i.e. of the phosphorus present in phosphonium groups, of less than 1% of phosphorus present in phosphonium groups, based on the total weight of the flame-retardant treated fabric. More precisely, it has now been found that, surprisingly, when the oxidation step (a3) is carried out in the presence of a metabisulfite salt used a pH of less than 4 (typically when the oxidation using H₂O₂ is followed by a treatment using a metabisulfite salt at a pH of less than 4, contrary to the usual conditions wherein metabisulfite salt is used as a scavenger but at a pH of at least 5, typically of at least 6), then the step (a) systematically leads to a trivalent phosphorous content of less than 1% (with sodium metabisulfite at a pH of about 2, this content is of about 0.8%). Therefore, when step (a) is conducted in these specific conditions, there is no need of step (b).

Accordingly, another specific subject matter of the instant invention is a process that directly allows to obtain a flame-retardant treated fabric according to the present invention, that contains less than 1% by weight, generally less than 0.9% by weight and in most cases less than 0.8% by weight of phosphorus present in phosphonium groups (trivalent phosphorus), based on the total weight of the flame-retardant treated fabric. This specific process, that do not need the implementation of a "checking" step (b) as defined above, contains a flame retardant treatment, including the following steps:
▪ step 1 : an impregnation of said fabric with the condensate of (i) a tetrakis (hydroxyorgano) phosphonium salt; and (ii) urea or thiourea , preferably followed by a drying
▪ step 2 : a curing with ammonia of the impregnated condensate ;
▪ step 3 : an oxidation of the polymer resulting from the curing, typically with H₂O₂ , said oxidation including and/or being followed by a treatment with a metabisulfite salt, preferably sodium metabisulfite, at a pH of below 4, preferably below 3, for example at a pH of 1.5 to 2.5, (e.g. from 1.8 to 2.2, typically of about 2).

Typically, in step 3, an oxidation is first carried out using hydrogen peroxide H₂O₂ or another oxidant, and then the treated fabric is treated with a metabisulfite salt, preferably sodium metabisulfite, at a pH of below 4, preferably 3, for example at a pH of 1.5 to 2.5, typically with SMBS at a pH of about 2.

Different features and specific embodiments of the invention are described in more details herein-after :
According to a first variant, the textile article of the invention is intended to be in indirect contact with the skin (namely with a layer of clothing between the treated surface and the skin). In that case, it is advantageous that it comprises less than 300 ppm, preferably less than 200 ppm of free formaldehyde, as measured according to the European standard No. EN ISO 14184-1.

According to a second variant, the textile article of the invention is a intended for direct contact with the skin. Then, it is highly preferable that it comprises less than 75 ppm of free formaldehyde , as measured according to the European standard No. EN ISO 14184-1.

According to a specific embodiment, the tetrakis (hydroxyorgano) phosphonium salt is tetrakis (hydroxyorgano) phosphonium chloride (THPC). Alternatively, it may be advantageous that the tetrakis (hydroxyorgano) phosphonium salt is tetrakis (hydroxyorgano) phosphonium sulfate (THPS)

The treated fabric advantageously comprises cellulosic fibers, for example natural cellulosic fibers such as fibers of cotton, linen, jute, or hessian ; or regenerated cellulosic material.

According to a specific embodiment, the treated fabric essentially comprises (typically for at least 95%) cellulosic fibers.

According to another embodiment, the fabric may comprise a mixture of cellulosic fibers together with non cellulosic fibers, said non cellulosic fibers being for example natural fibers such as wool or silk, or synthetic fibers such as polyester, polyamide, or aramid. As an example, the fabric may comprise a mixture of 60% cotton and 40% polyester.

The invention will now be further illustrated by the following illustrative example.

### Example 1

Two treated fabrics having a total content of phosphorus of 2% based on the total weight of the flame-retardant treated fabric have been compared :
**Fabric** 1 : **Comparative**
   containing trivalent phosphorus at a content more than 1% of based on the total weight of the flame-retardant treated fabric
**Fabric** 2 : **according to the invention**
   containing trivalent phosphorus at a content of 0.9% of based on the total weight of the flame-retardant treated fabric

The free HCOH content on the fabric has been measured and are reported in the table below :

| | Free HCOH content (pppm) | |
|---|---|---|
| time (years) | Fabric 1 (comparative) | Fabric 2 invention) |
| 0 | 100 | 100 |
| 0.5 | 125 | 100 |
| 1 | 150 | 100 |
| 2 | 205 | 100 |
| 3 | 305 | 100 |

### Example 2

In order to illustrate the advantages of the succession of step 1 to step 3 of the process of the invention, a comparison test has been conducted on fabric treated with PERFORM chemical, ammonia cured and oxidised with hydrogen peroxide according to the standard industry procedure, using sodium metabisulfite (SMBS) at a pH of 5, and the same but using sodium metabisulfite (SMBS) at a pH of 2

More precisely, a fabric treatment has been carried out as follows :
▪ ***Impregnation***
   514g of a fabric was immersed in a bath having the following composition: 481 g of PERFORM CC (available at Solvay) in 519 g of water as a solvent.
   The fabric was then immediately passed through a pad mangle and into an oven for drying at 120 °C for approximately 1 minute.
▪ ***Ammonia curing***
   The PERFORM CC treated fabric was then subjected to an ammonia atmosphere for 15 seconds by passing through an ammonia cure unit.
   After sampling this resulted in 577g of impregnated and cured fabric.
▪ ***H₂O₂ Oxidation***
   The 577g of cured fabric was then immersed for 10 minutes in a bath with the following composition: 2L of 35% hydrogen peroxide in 8L of water as a solvent.
   The fabric was then immersed for 15 minutes in another bath with the following composition: 100g of soda ash in 10L of water as a solvent.
   The fabric was then immersed for 45 minutes in another bath with the following composition: 10L of water.
   The fabric was then immersed for 5 minutes in another bath with the following composition: 10L of water, whereby a bulk oxidised fabric (BOF) is obtained.
▪ ***Sodium metabisulfite treatment***
   As a comparative test, a first sample (Sample 1) of the BOF as obtained after the treatment steps as defined above was treated at a pH of 5.
   As an illustration of the instant invention, the same treatment has been carried out on a second Sample of the BOF (Sample 2), in exactly the same conditions as for Sample 1, but with a treatment at a pH of 2.
      **Sample 1 (Comparative test)**
         13.4 g of the BOF (=Sample 1) was immersed in a bath with the following composition: 27.4g of 40% sodium metabisulfite in 1L of water as a solvent, with a resulting pH of 5, for 5 minutes at 70°C.
         Sample 1 was then immersed for 5 minutes in another bath with the following composition: 1L of water at 80°C
         Sample 1 was then immersed for 5 minutes in another bath with the following composition: 1L of water at 80°C
         Sample 1 was then immersed for 5 minutes in a bath with the following composition: 1L of water at 20°C.
      **Sample 2 (Illustrative)**
         13.9 g of the BOF (=Sample 2 ) was immersed in a bath with the following composition: 27.4g of 40% sodium metabisulfite plus 40g of 1M HCl in 1L of water as a solvent, with a resulting pH of 2 for 5 minutes at ~70°C.
         Sample 2 was then immersed for 5 minutes in another bath with the following composition: 1L of water at ~80°C
         Sample 2 was then immersed for 5 minutes in another bath with the following composition: 1L of water at ~80°C
         Sample 2 was then immersed for 5 minutes in another bath with the following composition: 1L of water at 20°C.
   As a result, a trivalent phosphorus_content content of less than 1% (0.84%) has been obtained when SMBS is used at pH=2 according to the invention (Sample 2).
   On the other hand, a content of more than 1% (1.26%) has been obtained in the standard conditions using SMBS is used (sample 1)
   With the content of less than 1% as obtained according to the invention, the free content of HCOH remains very low and stable over the time (Sample 2), when it increases with the time with the standard conditions of treatment (sample 1).

## Claims

1. A textile article comprising at least one flame-retardant treated fabric including an oxidized polymer obtained from an ammonia curing of a condensate of (i) a tetrakis (hydroxyorgano) phosphonium salt; and (ii) urea and/or thiourea ; followed by an oxidation into phosphine oxide groups of at least one part of the phosphonium groups present on the cured condensate,
wherein said flame-retardant treated fabric :
- is intended to be used as a stable substrate in which the formation of formaldehyde over the time is inhibited ; and
- contains less than 1% by weight of phosphorus present in phosphonium groups, based on the total weight of the flame-retardant treated fabric.

2. A textile article according to claim 1 wherein the flame-retardant treated fabric contains less than 0.9% by weight of phosphorus present in phosphonium groups, based on the total weight of the flame-retardant treated fabric.

3. A textile article according to claim 1 or 2 intended to an indirect contact with the skin, with a clothing between the treated surface and the skin, that comprises less than 300 ppm, preferably less than 200 ppm of free formaldehyde as measured according to the European Standard No. EN ISO 14184-1.

4. A textile article according to claim 1 or 2 intended to a direct contact with the skin, that comprises less than 75 ppm of free formaldehyde as measured according to the European Standard No. EN ISO 14184-1.

5. A textile article according to any of claim 1 to 4, wherein the tetrakis (hydroxyorgano) phosphonium salt is tetrakis (hydroxyorgano) phosphonium chloride (THPC)

6. A textile article according to any of claim 1 to 4, wherein the tetrakis (hydroxyorgano) phosphonium salt is tetrakis (hydroxyorgano) phosphonium sulfate (THPS)

7. A textile article according to any of claim 1 to 4, wherein the oxidized polymer is obtained from an ammonia curing of a condensate of (i) a tetrakis (hydroxyorgano) phosphonium salt; (ii) urea and/or thiourea, toogether with an an aliphatic amine having 12 carbon atoms or more; followed by an oxidation into phosphine oxide groups of at least one part of the phosphonium groups present on the cured condensate.

8. A process for preparing a textile article as defined in claim 1, comprising :
(a) a flame retardant treatment of the fabric, including :
(a1) an impregnation of said fabric with the condensate of (i) a tetrakis (hydroxyorgano) phosphonium salt; and (ii) urea or thiourea,
optionally together with an aliphatic amine having 12 carbon atoms or more
(a2) a curing with ammonia of the impregnated condensate ;
(a3) an oxidation of the polymer resulting from the curing, typically with H2O2
(b) an analysis of the content of the phosphonium groups in the fabric, for example by ³¹P NMR, followed by a repetition of the sequence of the steps (a3) and(b) if the analysis shows that the fabric contains 1% or more of phosphorus present in phosphonium groups, based on the total weight of the flame-retardant treated fabric.

9. The process of claim 8, wherein in step (b), the analysis is followed by a repetition of the sequence of steps (a3) and (b) if the analysis shows that the oxidized polymer contains 0.9% or more of phosphorus present in phosphonium groups, based on the total weight of the flame-retardant treated fabric.

10. A process for preparing a textile article as defined in claim 1, comprising the following steps :
▪ step 1 :
an impregnation of said fabric with the condensate of (i) a tetrakis (hydroxyorgano) phosphonium salt; and (ii) urea or thiourea
▪ step 2 :
a curing with ammonia of the impregnated condensate ;
▪ step 3 :
an oxidation of the polymer resulting from the curing, said oxidation including and/or being followed by a treatment with a metabisulfite salt at a pH of below 4, preferably below 3.

11. The use of a flame-retardant treated fabric as defined in any one of claim 1 to 7 or as obtained according to any of claim 6 to 10 as a substrate stabilized against formation of formaldehyde, for example for a long term contact with the skin.

12. Use according to claim 11, wherein the flame-retardant treated fabric is used for a long term contact with the skin, preferably more than one year, more preferably more than 2 years, and even more preferably at least 3 years, after the synthesis of the oxidized polymer

## Patentansprüche

1. Textilgegenstand, umfassend wenigstens ein flammhemmend behandeltes Gewebe, das ein oxidiertes Polymer enthält, erhalten durch eine Ammoniakhärtung eines Kondensats von (i) einem Tetrakis(hydroxyorgano)phosphoniumsalz; und (ii) Harnstoff und/oder Thioharnstoff; gefolgt von einer Oxidation wenigstens eines Teils der auf dem gehärteten Kondensat vorhandenen Phosphoniumgruppen zu Phosphinoxidgruppen,
wobei das flammhemmend behandelte Gewebe:
- zur Verwendung als stabiles Substrat vorgesehen ist, bei dem die Entstehung von Formaldehyd mit der Zeit gehemmt ist; und
- weniger als 1 Gew.-% Phosphor, der in Phosphoniumgruppen vorliegt, enthält, bezogen auf das Gesamtgewicht des flammhemmend behandelten Gewebes.

2. Textilgegenstand gemäß Anspruch 1, wobei das flammhemmend behandelte Gewebe weniger als 0,9 Gew.-% Phosphor, der in Phosphoniumgruppen vorliegt, enthält, bezogen auf das Gesamtgewicht des flammhemmend behandelten Gewebes.

3. Textilgegenstand gemäß Anspruch 1 oder 2, vorgesehen für einen indirekten Kontakt mit der Haut mit einem Kleidungsstück zwischen der behandelten Oberfläche und der Haut, umfassend weniger als 300 ppm, vorzugsweise weniger als 200 ppm, an freiem Formaldehyd, wie gemessen gemäß dem Europäischen Standard Nr. EN ISO 14184-1.

4. Textilgegenstand gemäß Anspruch 1 oder 2, vorgesehen für einen direkten Kontakt mit der Haut, umfassend weniger als 75 ppm an freiem Formaldehyd, wie gemessen gemäß dem Europäischen Standard Nr. EN ISO 14184-1.

5. Textilgegenstand gemäß einem von Anspruch 1 bis 4, wobei das Tetrakis(hydroxyorgano)phosphoniumsalz Tetrakis(hydroxyorgano)phosphoniumchlorid (THPC) ist.

6. Textilgegenstand gemäß einem von Anspruch 1 bis 4, wobei das Tetrakis(hydroxyorgano)phosphoniumsalz Tetrakis(hydroxyorgano)phosphoniumsulfat (THPS) ist.

7. Textilgegenstand gemäß einem von Anspruch 1 bis 4, wobei das oxidierte Polymer erhalten ist durch eine Ammoniakhärtung eines Kondensats von (i) einem Tetrakis(hydroxyorgano)phosphoniumsalz; (ii) Harnstoff und/oder Thioharnstoff zusammen mit einem aliphatischen Amin mit 12 oder mehr Kohlenstoffatomen; gefolgt von einer Oxidation wenigstens eines Teils der auf dem gehärteten Kondensat vorhandenen Phosphoniumgruppen zu Phosphinoxidgruppen.

8. Verfahren zur Herstellung eines Textilgegenstands gemäß Anspruch 1, umfassend:
(a) eine flammhemmende Behandlung des Gewebes, die einschließt:
(a1) eine Imprägnierung des Gewebes mit dem Kondensat von (i) einem Tetrakis(hydroxyorgano)phosphoniumsalz; und (ii) Harnstoff oder Thioharnstoff, gegebenenfalls zusammen mit einem aliphatischen Amin mit 12 oder mehr Kohlenstoffatomen,
(a2) eine Härtung des imprägnierten Kondensats mit Ammoniak;
(a3) eine Oxidation des durch die Härtung erhaltenen Polymers, typischerweise mit H2O2,
(b) eine Analyse des Gehalts an den Phosphoniumgruppen in dem Gewebe, beispielsweise durch ³¹P-NMR, gefolgt von einer Wiederholung der Abfolge der Schritte (a3) und (b), wenn die Analyse zeigt, dass das Gewebe 1 % oder mehr an Phosphor, der in Phosphoniumgruppen vorliegt, enthält, bezogen auf das Gesamtgewicht des flammhemmend behandelten Gewebes.

9. Verfahren gemäß Anspruch 8, wobei bei Schritt (b) die Analyse von einer Wiederholung der Abfolge der Schritte (a3) und (b) gefolgt wird, wenn die Analyse zeigt, dass das oxidierte Polymer 0,9 % oder mehr an Phosphor, der in Phosphoniumgruppen vorliegt, enthält, bezogen auf das Gesamtgewicht des flammhemmend behandelten Gewebes.

10. Verfahren zur Herstellung eines Textilgegenstands gemäß Anspruch 1, umfassend die folgenden Schritte:
• Schritt 1:
eine Imprägnierung des Gewebes mit dem Kondensat von (i) einem Tetrakis(hydroxyorgano)phosphoniumsalz; und (ii) Harnstoff oder Thioharnstoff
• Schritt 2:
eine Härtung des imprägnierten Kondensats mit Ammoniak;
• Schritt 3:
eine Oxidation des durch die Härtung erhaltenen Polymers, wobei die Oxidation eine Behandlung mit einem Metabisulfitsalz bei einem pH-Wert von unter 4, vorzugsweise unter 3, einschließt und/oder davon gefolgt wird.

11. Verwendung eines flammhemmend behandelten Gewebes gemäß einem von Anspruch 1 bis 7 oder erhalten gemäß einem von Anspruch 6 bis 10 als Substrat, das gegen Entstehung von Formaldehyd stabilisiert ist, beispielsweise für einen Langzeitkontakt mit der Haut.

12. Verwendung gemäß Anspruch 11, wobei das flammhemmend behandelte Gewebe für einen Langzeitkontakt mit der Haut verwendet wird, vorzugsweise mehr als ein Jahr, bevorzugter mehr als 2 Jahre und noch bevorzugter wenigstens 3 Jahre nach der Synthese des oxidierten Polymers.

## Revendications

1. Article de textile comprenant au moins un tissu traité par un retardateur de flamme comprenant un polymère oxydé obtenu à partir d'un durcissement à l'ammoniac d'un condensat de (i) un sel de tétrakis(hydroxyorgano)phosphonium ; et (ii) une urée et/ou une thiourée ; suivi par une oxydation en groupements oxyde de phosphine d'au moins une partie des groupements phosphonium présents sur le condensat durci,
ledit tissu traité par un retardateur de flamme :
- étant destiné à être utilisé en tant que substrat stable dans lequel la formation de formaldéhyde dans le temps est inhibée ; et
- contenant moins de 1 % en poids de phosphore présent dans des groupements phosphonium, sur la base du poids total du tissu traité par un retardateur de flamme.

2. Article de textile selon la revendication 1, dans lequel le tissu traité par un retardateur de flamme contient moins de 0,9 % en poids de phosphore présent dans des groupements phosphonium, sur la base du poids total du tissu traité par un retardateur de flamme.

3. Article de textile selon la revendication 1 ou 2 destiné à un contact indirect avec la peau, avec un vêtement entre la surface traitée et la peau, qui comprend moins de 300 ppm, préférablement moins de 200 ppm de formaldéhyde libre comme mesuré selon la norme européenne n° EN ISO 14184-1.

4. Article de textile selon la revendication 1 ou 2 destiné à un contact direct avec la peau, qui comprend moins de 75 ppm de formaldéhyde libre comme mesuré selon la norme européenne n° EN ISO 14184-1.

5. Article de textile selon l'une quelconque des revendications 1 à 4, dans lequel le sel de tétrakis(hydroxyorgano)phosphonium est le chlorure de tétrakis(hydroxyorgano)phosphonium (THPC).

6. Article de textile selon l'une quelconque des revendications 1 à 4, dans lequel le sel de tétrakis(hydroxyorgano)phosphonium est le sulfate de tétrakis(hydroxyorgano)phosphonium (THPS).

7. Article de textile selon l'une quelconque des revendications 1 à 4, dans lequel le polymère oxydé est obtenu à partir d'un durcissement à l'ammoniac d'un condensat de (i) un sel de tétrakis(hydroxyorgano)phosphonium ; (ii) une urée et/ou une thiourée, conjointement avec une amine aliphatique ayant 12 atomes de carbone ou plus ; suivi par une oxydation en groupements oxyde de phosphine d'au moins une partie des groupements phosphonium présents sur le condensat durci.

8. Procédé pour la préparation d'un article de textile tel que défini dans la revendication 1, comprenant :
(a) un traitement du tissu par un retardateur de flamme, comprenant :
(a1) une imprégnation dudit tissu avec le condensat de (i) un sel de
tétrakis(hydroxyorgano)phosphonium ; et (ii) une urée ou une thiourée, optionnellement conjointement avec une amine aliphatique ayant 12
atomes de carbone ou plus
(a2) un durcissement avec de l'ammoniac du condensat imprégné ;
(a3) une oxydation du polymère résultant du durcissement, typiquement avec H2O2
(b) une analyse de la teneur des groupements phosphonium dans le tissu, par exemple par RMN du ³¹P, suivie par une répétition de la séquence des étapes (a3) et (b) si l'analyse montre que le tissu contient 1 % ou plus de phosphore présent dans des groupements phosphonium, sur la base du poids total du tissu traité par un retardateur de flamme.

9. Procédé selon la revendication 8, dans lequel dans l'étape (b), l'analyse est suivie par une répétition de la séquence des étapes (a3) et (b) si l'analyse montre que le polymère oxydé contient 0,9 % ou plus de phosphore présent dans des groupements phosphonium, sur la base du poids total du tissu traité par un retardateur de flamme.

10. Procédé pour la préparation d'un article de textile tel que défini dans la revendication 1, comprenant les étapes suivantes :
• étape 1 :
une imprégnation dudit tissu avec le condensat de (i) un sel de tétrakis(hydroxyorgano)phosphonium ; et (ii) une urée ou une thiourée
• étape 2 :
un durcissement avec de l'ammoniac du condensat imprégné ;
• étape 3 :
une oxydation du polymère résultant du durcissement, ladite oxydation incluant et/ou étant suivie par un traitement par un sel de métabisulfite à un pH de moins de 4, préférablement de moins de 3.

11. Utilisation d'un tissu traité par un retardateur de flamme tel que défini dans l'une quelconque des revendications 1 à 7 ou tel qu'obtenu selon l'une quelconque des revendications 6 à 10 en tant que substrat stabilisé contre la formation de formaldéhyde, par exemple pour un contact à long terme avec la peau.

12. Utilisation selon la revendication 11, dans laquelle le tissu traité par un retardateur de flamme est utilisé pour un contact à long terme avec la peau, préférablement de plus d'une année, plus préférablement de plus de 2 ans, et encore plus préférablement d'au moins 3 ans, après la synthèse du polymère oxydé.
